

July 23, 1946.

I. G. NIXON

2,404,452

## PRODUCTION OF AVIATION GASOLINE

Filed March 27, 1944



Inventor: Ivor G. Nixon

By his Attorney: John H. Morris

## UNITED STATES PATENT OFFICE

2,404,452

## PRODUCTION OF AVIATION GASOLINE

Ivor G. Nixon, Ewell, England, assignor to Shell Development Company, San Francisco, Calif., a corporation of Delaware

Application March 27, 1944, Serial No. 528,290

14 Claims.

(Cl. 196—49)

1

This invention relates to the manufacture of aviation gasoline base stocks by the cracking and re-cracking of selected hydrocarbon distillates, and especially to the art of re-forming low octane naphthas to increase their rich mixture ratings in blends in super-charged aviation engines. These ratings are expressed in "index numbers" which are obtained by calculation from blends tested at their detonation limited power outputs in a Cooperative Fuel Research Committee (C. F. R.) super-charged 3-C engine. The test was carried out according to the Coordinating Research Council method designated CRC-F-4-443, and described in the report of August 2, 1943 of the subcommittee on Blending Octane Numbers of the Aviation Gasoline Advisory Committee to the Petroleum Administrator for War. Index numbers are approximately equal to the percent of power that the fuel can produce as compared with the power produced by iso-octane under the same conditions.

"Index number" differs from "octane number" in that the former is a measure of the allowable output of a super-charged aviation engine under take-off and climb conditions while octane number is a measure of the detonation tendency of the fuel in a non-super-charged engine under cruising conditions. Thus octane numbers and index numbers refer to very different fuel properties.

It is well known that naphthas used in the blending of high grade motor fuels, and particularly aviation gasoline, must have a high anti-knock value, must be free of gum-forming components, and must maintain their anti-knock properties under severe engine conditions, i. e. high temperature, high compression and rich mixture. For these reasons naphthas rich in aromatic hydrocarbons and substantially free from olefins are preferred. Aromatics are known to have excellent anti-knock properties which do not decrease under severe operating conditions and have no tendency to form gums or to deteriorate otherwise during storage. Olefins, on the contrary, frequently oxidize and polymerize during storage, forming gums, and thus render a motor fuel less desirable for airplane engines.

It is well known that by suitable thermal treatments which may involve carbon-carbon scission and dehydrogenation or isomerization or polymerization or a combination of these reactions, it is possible to increase the octane number and the aromatic content of hydrocarbon oils without substantially changing their boiling range. At the same time, however, such thermal operations,

2

when conducted by conventional methods, usually cause the formation of large amounts of olefins. For this reason, thermally cracked naphthas have not generally been used in aviation gasolines.

It is also known that for a given hydrocarbon feed, a practical limit is placed on the attainable severity of cracking conditions because of coke deposition. There is a certain severity of cracking above which coking becomes very rapid, and below which it is very slow. This critical value may to some extent depend upon the design of the furnace in which the cracking is conducted, but for a given furnace it is a function of the nature of the feed. Since a furnace must be shut down and cleaned as soon as deposition of coke begins to plug it, it is obvious that only processes in which coking is relatively slow are economically practical. However, more severe cracking conditions can be maintained without objectionable coking by any one or more of the following methods: (1) introducing into the cracking zone, together with the naphtha, low boiling hydrocarbons containing from 1 to about 5 carbon atoms per molecule; (2) reducing the amount of olefins present in the naphtha to be cracked; and (3) increasing the aromatic content of the fraction to be cracked.

It has been discovered that if certain selected naphtha fractions having low olefin content are cracked and re-cracked under certain conditions, a relatively high boiling fraction may be obtained that has a high concentration of aromatics, a low concentration of olefins and a greatly increased index number.

It is an object of the present invention to provide an improved method for making aviation blending stock having a high rich mixture rating in supercharged engines, that is, a blending stock having a high index number. It is another object to produce naphtha having superior anti-knock and storage properties. Another object is to provide a cracking process capable of producing a naphtha having high aromatic content and unusually low olefin content from which pure aromatics, particularly toluene, may be obtained, if desired. Still another object is to produce a maximum amount of aromatics and high index number components from a naphtha fraction with a minimum amount of re-forming capacity.

The process of this invention comprises the following essential steps:

1. Thermally cracking a straight run naphtha having a selected boiling range;

2. Fractionating the resulting cracked products to obtain a selected naphtha fraction;

3. Re-cracking said second fraction, preferably in the presence of a light feed;

4. Fractionating the resulting re-cracked products to produce light aviation blending stock and a relatively heavy fraction boiling essentially within about 140° and 225° C.;

5. Further re-cracking said heavy fraction, preferably in the presence of a light feed; and

6. Fractionating the resulting cracked heavy fraction to produce a heavy aviation blending stock of high index number.

In addition to these essential steps, there may be inserted between steps 4 and 5 a treating step wherein both the light and heavy fractions are treated to remove small quantities of olefins which may be present before they are separated. Further, the final heavy aviation base stock may be fractionated and treated to improve its aviation blending characteristics.

"Thermal" cracking means non-catalytic cracking or cracking in the absence of a catalyst as understood in the conventional sense, in accordance with the accepted usage in the prior art as exemplified by the definition found on page 37 of "The Chemistry of Petroleum Derivatives" by Carlton Ellis, published in 1934.

The success of the present invention, and particularly of the re-cracking, depends on the proper selection of the straight run and the cracked naphtha fractions. It is only when all three of these fractions are properly chosen and cracked under the proper conditions that the full benefits of this invention are obtained.

The nature of the invention will be better understood from the following detailed description, taken together with the drawing forming a part of this specification. This drawing presents a simplified flow diagram of a preferred embodiment of the invention.

For simplicity the drawing does not show pumps, heat exchangers, valves, by-passes, vents, reboilers, condensers, and other auxiliaries, the proper placement of which will at once be evident to those skilled in the art.

The straight run hydrocarbon naphtha which forms the starting material of the present process may originate from any crude, though aromatic or naphthenic oils are preferred to paraffinic ones. For instance, a straight run naphtha fraction having a U. O. P. characterization factor below 11.6 and preferably below 11.4 is preferred. The U. O. P. characterization factor is a measure of the paraffinicity of an oil. A highly paraffinic oil has a factor of 12.5 and a highly aromatic and naphthenic oil has a lower factor approaching 10 as a minimum. (See "Characterization of petroleum fractions" by Watson, Nelson and Murphy of U. O. P., Ind. and Eng. Chem., vol. 27, No. 12, p. 1460.)

Furthermore, this starting material or first naphtha fraction should preferably have an A. S. T. M. initial boiling point of not below 90° C. and preferably not below 100° C. Its end boiling point by A. S. T. M. distillation should be below about 230° C. and preferably below about 200° C. The reasons for these limitations are as follows: first, most of the hydrocarbons boiling outside these limits tend upon cracking to produce relatively large amounts of olefins boiling within the boiling range of the cracked naphtha selected for the subsequent cracking steps and second, that this fraction contains most of the aromatic hydrocarbons which are valuable for aviation fuel blend-

ing stocks or which yield such aromatics in the subsequent cracking steps of the process. If the cracking stock is very rich in olefins, then the product of re-cracking, that is the aviation blending stock, will also be relatively rich in olefins. Also more coke formation will be encountered which will, in part, limit the index number that can be obtained in the process. That this must be avoided has been pointed out before.

Thus the boiling range of this starting material lies in a range essentially within about 90° and 230° C. If the boiling range is high, say essentially within about 150° and 230° C., an increase in the yield of the heavy aviation blending stock is obtained at the expense of a decrease in the yield of the light aviation blending stock which may be removed between steps 4 and 5, mentioned above. For example, if the initial boiling point of the starting material is above the boiling point of toluene, say at about 110° C., then the yield of the heavy aviation blending stock is almost twice that compared to the yield obtained from a starting material having an initial boiling point at 95° C. and including toluene, while the total yield of light and heavy aviation fraction remains about the same.

In the first step of this process, the selected straight run naphtha fraction is introduced through line 11 into a cracking zone such as a cracking coil 19 wherein it is cracked in a pseudo liquid phase (that is, cracked above the critical temperature and pressure of the naphtha fraction) under conditions as severe as is practical without excessive coking. If desired, the time of cracking may be extended and controlled with the aid of a reaction or soaking chamber not shown. For instance, these cracking conditions have been found to correspond to cracking temperatures between about 540° C. and 580° C. and inlet pressures between about 40 and 100 kg./sq. cm.

In the second step, the resulting cracked products from zone 18 are withdrawn through line 12 and are quenched and fractionally distilled in the distillation column 20 to separate therefrom those products boiling above about 230° C. and preferably above 200° C. which are withdrawn from the bottom of the column 20 through line 21. The remaining lighter portion of the products is withdrawn from the top of the column through line 22 and introduced into another fractional distillation column 25 wherein the products boiling below about 90° C. and preferably below about 100° C. are withdrawn through vapor line 26 at the top of column 25. The remaining fraction, which has a boiling range essentially within about 90° C. and 230° C. will be referred to hereinafter as the "second naphtha fraction," and is withdrawn from the bottom of column 25 through line 27.

The gases and light hydrocarbons withdrawn from the top of column 25 through line 26 may be separated and employed in other processes. For example, the C<sub>5</sub> and lighter hydrocarbons may be alkylated to produce a blending stock for gasoline, or any C<sub>5</sub> or higher hydrocarbons may be employed as a blending stock for motor gasolines if desired. The C<sub>4</sub> hydrocarbons may be converted into octylenes, cracked to produce butadiene, or alkylated to produce aviation blending stocks. The C<sub>3</sub> hydrocarbons may be chemically treated to produce acetone; and the C<sub>1</sub> and C<sub>2</sub> hydrocarbons may be employed as fuel. Still further, the hydrocarbons having from 3 to 5 carbon atoms per molecule may be employed again in this process as the light feed that is preferably introduced

into the next two cracking steps as described below.

This second naphtha fraction usually has an octane number of at least 74 or 75, and can be used with advantage as a motor fuel, but not as aviation fuel. It is characterized by a relatively high content of monocyclic aromatics and naphthenes, as opposed to naphthas boiling above about 230° C., which contain a relatively large amount of polycyclic aromatics and naphthenes. These latter compounds should not be included in the selective fraction because upon cracking under severe conditions they tend to promote coke formation and lower the quality of the final product. Moreover, as pointed out before, relatively high boiling hydrocarbons tend to form large amounts of olefins upon cracking, which boil within gasoline boiling range.

By further treating this second naphtha fraction as described below, its octane number can be greatly improved, its aromatic content increased, and its paraffin, naphthene, and particularly olefin content decreased so that it can be used for aviation fuel.

In the third step, the second naphtha fraction is introduced into a second cracking coil 30 through line 31, wherein it is re-cracked under conditions similar to those maintained in cracking zone 10. It is desirable, although not necessary, to add to this second naphtha fraction, through valved line 32 before it enters zone 30, a minor amount of light hydrocarbon feed consisting essentially of at least one hydrocarbon having from 1 to 5 and preferably from 3 to 5 carbon atoms per molecule. The amount of the light feed employed as previously indicated is merely sufficient to reduce the speed of coking for economical purposes, and otherwise has no material effect on the properties of the selected cracked naphtha fractions. This amount may vary between about 5 and 30% and preferably between 5 and 15% by volume of the feed to zone 30.

The re-cracking operation in zone 30 should be conducted under the most severe conditions which can be tolerated without excessive coking. These conditions may be more severe than those in the first cracking zone 1 because many components of the original fuel, which tend to decompose readily, and cause coking, have been cracked in the first cracking step and eliminated in the fractional distillation columns 20 and 25. The conditions correspond, for example, to temperatures ranging between about 540°-580° C. and pressures ranging between about 40 and 100 kgs./cm.<sup>2</sup>. The resulting re-cracked products are withdrawn through line 33, quenched, and fractionated as described in the second step.

The severity of the cracking may be defined either by the cracking conditions, or by the changes brought about by these cracking conditions in the properties of the hydrocarbon and particularly in its boiling range. The latter method is particularly applicable when the feed stock has a relatively narrow boiling range, because in such a case, portions whose boiling ranges are changed are most likely to boil outside the boiling limits of the feed. When defined according to this method, the cracking conditions which, for this process, are such that a cracked fraction having the same boiling range as the naphtha feed amounts to about 50% to 90% of the cracked products in each cracking operation, and preferably about 70% in the first operation and about 60% in

the second operation. In the third cracking operation, the change in boiling range is less significant because of its relatively high aromatic content.

Another way of determining the severity of cracking includes methods of determining the aromatic content of the cracked product. Some of the ways of measuring this aromatic content are as follows:

One method is by measuring the change in octane rating of the fraction after it is cracked. In general, the octane rating is determined for a debutanized fraction having an end point of 200° C. For example, the second naphtha fraction produced in the process of this invention should preferably have an octane number of between 74 and 78 by the C. F. R. motor method.

Another method is by measuring the aromatic content by percent by weight of the cracked product which is extractable in 98% sulfuric acid.

This method is not very accurate, because the strong acid tends to polymerize some of the olefins, causing them to remain in the oil phase. However, if the bromine number of the cracked product is below about 10, the weight percent extractable is within about 5% of the amount of aromatics present in the cracked product.

A more accurate method is by means of the specific dispersion which is a measure of the percentage of aromatics in the resulting product (see Ind. and Eng. Chem., vol. 29, No. 3, March, 1937, pp. 319-325). For example, a fraction which has a specific dispersion of about 135 contains at least about 50% aromatics. Thus, the selected third naphtha fraction obtained from the products of zone 30 should have a specific dispersion of at least about 135 and preferably at least about 140.

It is essential that each cracking operation described in this process be carried out as a separate step. If it were attempted to maintain cracking conditions sufficiently severe to produce the desired result in one operation without intermediate separation of light and heavy components, heavy and tarry components produced in the initial stages would cause rapid coking in the subsequent stages. Moreover, the light unsaturated components formed at the beginning would be present in a large concentration, would polymerize to form olefins boiling within the naphtha range, and thus would produce finally a more unsaturated naphtha, which is not desired.

In the fourth step, the cracked product from line 33 is introduced into the fractional distillation column 40 wherein the products boiling above about 230° C., and preferably above 200° C., are removed through bottom line 41 and the remaining portion is withdrawn through top line 42 into the fractionating column 45, wherein the lighter hydrocarbons boiling below about 90° C., and preferably below 100° C., are withdrawn through vapor line 46 to produce the "third naphtha fraction" which is withdrawn through bottom line 47.

This third naphtha fraction has an olefin content much lower and an aromatic content much higher than that of the corresponding fraction obtained from the products of the first cracking zone 10. This third fraction should have an octane number, by the C. F. R. motor method, at least 5 points higher than the second naphtha fraction present in line 27, and preferably should have an octane number between about 80 and 85. It should be between about 50 and 75% by weight extractable with strong sulfuric acid and should

have a specific dispersion of at least 140 and preferably 150 or above.

In a preferred, although not essential embodiment of this process, the third naphtha fraction is subjected to a refining treatment. Thus, as illustrated in the drawing, the third naphtha fraction from the bottom of column 45 is passed through lines 47 and 51 to a treating unit 50.

The type of treatment employed depends largely upon the properties of the third naphtha fraction. For instance, if this fraction should contain considerable amounts of olefins, a treatment adapted to remove the major part of the olefins is preferred. Such a treatment, for example, is a light sulfuric acid treatment. Although a sulfuric acid treatment is known ordinarily to reduce the octane number of cracked gasoline, it does, on the contrary, further raise the octane number of the third naphtha fraction prepared according to this invention. A suitable sulfuric acid treatment may involve the contact of the fraction with between about 1 and 5% by volume of a 95 to 98% sulfuric acid. The acid employed in the treating may be fresh or may be spent alkylation acid.

Other treatments which may be employed in the treating unit include for example passing the fraction over adsorption agents such as clay, bauxite, fuller's earth, diatomaceous earth, silica gel, etc., at elevated temperatures below incipient cracking; contacting with phosphoric acid of suitable concentration to produce a sludge containing the undesirable constituents which can be separated; selective hydrogenation in the presence of a suitable hydrogenation catalyst, such as finely divided nickel, chromium oxide, molybdenum or tungsten sulfide or a combination of these, etc.; treatment with catalyst of the clay type under conditions which do not cause substantial cracking; destruction or removal of harmful sulfur compound by doctor treatment, extraction with alkaline solution in the presence of a solutizer for mercaptans, or oxidation in the presence of copper catalysts, etc.

The specific conditions involved in the treating processes as above mentioned may be readily obtained from the book, "Chemical Refining of Petroleum," Kalichevsky and Stagner, published by Reinhold Publishing Corporation, 1942. In this book are descriptions of processes for the treatment of hydrocarbons with sulfuric acid (see Chapter II), with alkaline reagents (see Chapter IV), sweetening processes (see Chapter V), refining by adsorption (see Chapter VI) and refining with a solvent (see Chapter VII).

These treatments may be relatively light, i. e. much lighter than treatments which would have to be applied to conventionally cracked naphthas or to the naphtha obtained in the first cracking step of this process, in order to obtain a product having the same color, stability, low degree of unsaturation and low mercaptan content.

The treated naphtha may be redistilled in column 55 to remove higher boiling constituents formed during the treating operations which are withdrawn through bottom line 56. These bottoms from the re-distillation are usually highly aromatic and may be blended into fuel oils.

If desired, the untreated third naphtha fraction, or the treated and re-distilled naphtha fraction may be withdrawn through valved lines 48 or 57 and 52 to the toluene recovery plant 53, wherein toluene is extracted and withdrawn through valved line 54. The remaining non-toluene portion of the third naphtha fraction is returned to the process through valved line 58.

A portion of the third naphtha fraction (treated or untreated, and/or containing toluene or not) may, however, be removed from the system through valved line 59 and employed as an aviation blending stock, in that it now has an octane number between about 80 and 85 and an index number, in a blend with 4 cc. of tetra ethyl lead/gallon, between about 125 and 135.

Continuing the operation of the process of this invention, the untreated, or preferably the treated third naphtha fraction is passed into the fractionating column 60 through valved line 61, wherein it is separated into a light aviation base stock and a heavy fraction. The cut point for this separation may range essentially within about 140° and 155° C., but preferably wherein the xylenes and cumene which have high index numbers, pass overhead into the light aviation base stock (for instance, at about 150 or 152° C.). This light aviation base stock is withdrawn through vapor line 62 and if desired may be further treated or may be blended directly into aviation or other motor fuels.

The light aviation base stock should have an octane number by the C. F. R. motor method between about 80 and 85 and should have an index number in a blend with 4 cc. of tetra ethyl lead of between about 130 and 140. Between about 50 and 75% of the light aviation base stock should be extractable with strong sulfuric acid, and it should have a specific dispersion above about 140 and preferably above 150. The boiling range of this base stock may lie between about 90 and 155° C. and preferably between 100 and 150° C., although its end boiling point may be as low as 140° C.

The heavy naphtha fraction withdrawn from the bottom of column 60, which has a boiling range essentially within about 140 and 230° C. and preferably essentially within about 150 and 200° C., usually has an octane number by the C. F. R. motor method within about 80 and 85, but its index number in a blend with 4 cc. of tetra ethyl lead is usually much lower than that of the light aviation base stock withdrawn from the top of column 60. This heavy aviation base stock usually has an index number ranging only between about 110 and 125. The aromatic content of this heavy fraction from the bottom of column 60 is much higher than that of the light aviation base stock, in that it has a specific dispersion of at least 150 and preferably above and it is between 65 and 95% extractable with strong sulfuric acid.

In the fifth essential step, the heavy fraction withdrawn from the bottom of column 60 through lines 63 and 71 is introduced into a third cracking coil 70. As in cracking zone 30, it is also desirable, but not necessary, to introduce with the heavy fraction in line 63 a light hydrocarbon through valve line 72 consisting essentially of at least one hydrocarbon having preferably from 3 to 5 carbon atoms per molecule. The amount of this added light hydrocarbon should range between about 5 and 30% by volume, and preferably between about 5 and 15% by volume of the feed to cracking zone 70.

It is possible, but not preferred economically, to employ the treated third naphtha fraction from line 61 as the feed to cracking zone 70 by by-passing the column 60 through line 73.

The cracking in zone 70 is generally carried out under substantially the same conditions as those employed in zones 10 and 30, although

the pressure may be higher, if desired, ranging between about 40 and 95 kg./sq. cm.

In the sixth essential step, the resulting cracked heavy fraction is introduced into a fractionating column 80 through line 81 from cracking zone 10, wherein the products boiling above about 200° C. and preferably above about 180° C. are withdrawn through bottom line 82. The lower boiling fraction withdrawn through line 83 is distilled in fractionating column 85 to produce a 10 hydrocarbon fraction boiling below about 100° C. and preferably 120° C. withdrawn through top vapor line 86, and an intermediate fraction withdrawn through bottom line 87. This bottom product is a heavy aviation base stock usually 15 having an octane number above about 80 and an index number in a blend containing 4 cc. of tetra ethyl lead/gallon, between about 150 and 165. The index number range is considerably 20 higher than the index number of the light aviation base stock removed from the top of column 60, or the third naphtha fraction removed from line 59 or the heavy fraction in line 63.

The lighter hydrocarbon withdrawn through lines 46 and 86 of columns 45 and 85 may be 25 joined with those from the top of column 25 in line 26 and separated for use in the same manner as those described from line 26.

The heavier fractions withdrawn from lines 21, 41 and 82 of columns 20, 40 and 80, respectively, 20 are highly aromatic and may be blended, if desired, into fuel oils or used for any other suitable purposes.

The heavy aviation base stock may be withdrawn from the system through valve line 88 or 35 it may be subjected to treatment similar to that described for treating unit 50. If the heavy base stock is treated, it is passed through valve line 89 into the treating unit 90 and then passed into the re-run column 95 similar to column 55. 40 This treatment of the base stock does not materially change its octane number or its index

etc. Many of these blending agents may be obtained or produced from the by-products of this process.

It may be noted that the described process provides for the manufacture of a superior aviation base stock and valuable products from naphtha fractions of relatively little value.

The following comparative examples illustrate the invention:

#### Example I

A straight run naphtha fraction having the properties disclosed in the table below was cracked in a first cracking zone having a transfer temperature of about 548° C. and an inlet pressure of about 51 kg./sq. cm. to produce a cracked product which was fractionated to obtain a second naphtha fraction having the properties disclosed in the table below. This second naphtha fraction and a mixture of C<sub>3</sub> to C<sub>5</sub> cut amounting to about 14% of the feed was then cracked in a second cracking furnace having a transfer temperature of about 541° C. and an inlet pressure of about 63 kg./sq. cm. to produce a re-cracked product which was fractionated to obtain a third naphtha fraction having the properties disclosed in the table below. This third naphtha fraction was then acid treated with about 2% by weight of 98% sulfuric acid and re-distilled to remove any high polymers formed during the acid treatment. This treated fraction was then further fractionated into a light aviation base stock and a heavy fraction having the properties disclosed in the table below. The resulting heavy fraction and a mixture of C<sub>3</sub> and C<sub>5</sub> gases amounting to about 11% of the feed was then passed through a third cracking furnace having a transfer temperature of about 545° C. and an inlet pressure of about 76 kg./sq. cm. to produce a cracked product which was fractionated to obtain a heavy aviation base stock having the properties disclosed in the table below.

|                                                                   | Straight run naphtha fraction | Second naphtha fraction | Third naphtha fraction | Light aviation base stock | Heavy fraction | Heavy aviation base stock |
|-------------------------------------------------------------------|-------------------------------|-------------------------|------------------------|---------------------------|----------------|---------------------------|
| Specific gravity                                                  | 0.786                         | 0.807                   | 0.824                  | 0.805                     | 0.844          | 0.858                     |
| A. S. T. M.:                                                      |                               |                         |                        |                           |                |                           |
| I. B. P.:                                                         |                               |                         |                        |                           |                |                           |
| °C.                                                               | 120                           | 77                      | 110                    | 97                        | 146            | 130                       |
| °O.                                                               | 134                           | 123                     | 121                    | 108                       | 154            | 148                       |
| 10%                                                               |                               |                         |                        |                           |                |                           |
| °C.                                                               | 157                           | 146                     | 139                    | 117                       | 160            | 157 <sup>1/2</sup>        |
| 50%                                                               |                               |                         |                        |                           |                |                           |
| °C.                                                               | 210                           | 209                     | 166                    | 138                       | 170            | 169 <sup>1/2</sup>        |
| 90%                                                               |                               |                         |                        |                           |                |                           |
| F. B. P.                                                          |                               |                         |                        |                           |                |                           |
| °C.                                                               |                               | 180                     | 152                    | 179                       | 179            | 180                       |
| Bromine number                                                    | 9                             | 25.4                    | 6                      | 6 <sup>1/2</sup>          | 5              | 4                         |
| Percent by w. extractable with 98% H <sub>2</sub> SO <sub>4</sub> | 18                            | 49                      | 60                     | 53                        | 69             | 86                        |
| (Reed.) vapor pressure                                            |                               |                         | .8                     | 1.2                       | 0.3            | 0.4                       |
| Octane number (clear, A. S. T. M.—C. F. R. motor method)          | 52.6                          | 75.8                    | 81.5                   | 80.5                      | 83.5           | 190                       |
| Index number (in blends containing 4 cc. TEL)                     |                               |                         | 129                    | 136                       | 119            | 157                       |

<sup>1</sup> In a blend.

number from what it was before the treatment. 60

The treated product may be withdrawn from the top of column 95 through valve line 96 or it may be passed through valve line 97 into a blending plant 100 where it is mixed with other base stocks to produce a finished aviation gasoline. 65

Some suitable blending agents to produce a finished aviation gasoline include light straight run gasolines, isopentane, cyclopentane, neo-hexane, 2, 3-dimethyl butane, di-isopropyl ether, triptane, iso-octane, alkylation gasoline produced by reacting isobutane with C<sub>5</sub> and lower olefins, etc. These blending agents give the proper boiling range to the final blend and its octane number may be further improved by the addition of tetra-ethyl lead, aromatic mono-cyclic amines, 70 75

From the above table, it may be seen that the index number of the heavy aviation base stock is materially above that of the third naphtha fraction or even the light aviation base stock. Furthermore, it may be seen that the high boiling range of the heavy aviation base stock lends itself well for blending with iso-pentane and similar volatile blending stocks.

#### Example II

Another sample of a heavy fraction which had been cracked, fractionated, re-cracked and further fractionated as described in Example I had the properties shown in the table below. A feed consisting of this heavy fraction contained 13% by volume of a light hydrocarbon feed consisting

predominantly of propane and propylene, but also including some C<sub>4</sub> and C<sub>5</sub> hydrocarbons, was further cracked in a cracking coil at a temperature of about 540° C. and an inlet pressure of 76 kg./sq. cm. The resulting cracked product was then fractionated to obtain a heavy aviation gasoline base stock having the improved properties shown in the table below. It should be noted that the index number of the heavy aviation base stock is better than iso-octane containing 4 cc. tetra ethyl lead. The resulting cracked product was then fractionated to obtain a heavy aviation gasoline base stock having the improved properties shown in the table below.

|                                                                   | Heavy fraction | Heavy aviation base stock |
|-------------------------------------------------------------------|----------------|---------------------------|
| Specific gravity                                                  | 0.847          | 0.858                     |
| A. S. T. M.:                                                      |                |                           |
| I. B. P. ° C.                                                     | 149            | 133                       |
| 10% ° C.                                                          | 155            | 148                       |
| 50% ° C.                                                          | 162            | 158                       |
| 90% ° C.                                                          | 174.5          | 170.5                     |
| F. B. P. ° C.                                                     | 186            | 184                       |
| Bromine number                                                    | 4.7            | 3.5                       |
| Percent by w. extractable with 98% H <sub>2</sub> SO <sub>4</sub> | 68             | 87.0                      |
| (Reed.) vapor pressure                                            |                |                           |
| Octane number (clear, A. S. T. M.—C. F. R. motor method)          | 83.5           | 91.3                      |
| Index number (in blends containing 4 cc. TEL)                     |                | Above 154                 |

I claim as my invention:

1. A process for producing an aviation gasoline base stock from a straight run naphtha having a boiling range essentially within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction, separating the resulting re-cracked product by itself to produce a heavy fraction boiling between about 140° C. and about 230° C., further non-catalytically cracking said heavy fraction and separating the resulting further cracked product by itself to produce an aviation base stock boiling essentially within the range of about 100° C. and 200° C., each of said cracking operations being conducted at a temperature between about 540° C. and 580° C. and at a pressure between about 40 and 100 kg./sq. cm.

2. The process of claim 1, wherein the first cracking operation is conducted under conditions to yield a gasoline having an octane number above about 74 and said second cracking operation is conducted to yield a gasoline having an octane number above about 80.

3. The process of claim 1, wherein the naphtha fractions boil essentially within the range of about 100° C. and 200° C.

4. The process of claim 1, wherein said straight run naphtha fraction has a U. O. P. characterization factor below 11.6.

5. A process for producing an aviation gasoline base stock from a straight run naphtha having a boiling range within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction in the presence of a minor amount of a light feed consisting essentially of at least one hydrocarbon having from 3 to 5 carbon atoms per molecule, separat-

ing the resulting re-cracked product by itself to produce a heavy fraction boiling essentially within the range of about 140° C. and 230° C., further non-catalytically cracking said heavy fraction in the presence of a minor amount of a light feed consisting essentially of at least one hydrocarbon having from 3 to 5 carbon atoms per molecule, separating the resulting further cracked product by itself to produce an aviation base stock boiling essentially within the range of about 100° C. and 200° C., each of said cracking operations being conducted at a temperature between about 540° C. and 580° C. and at a pressure between about 40 and 100 kg./sq. cm.

6. The process of claim 5, wherein the amount of said light feed is between about 5 and 30% by volume of the fraction being cracked.

7. The process of claim 5, wherein said light feed is between about 5% and 15% by volume of the fraction being cracked.

8. A process for producing an aviation gasoline base stock from a straight run naphtha having a boiling range essentially within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction, separating the resulting re-cracked product by itself to produce a third naphtha fraction boiling essentially within the range of about 100° C. and 200° C., further separating said third naphtha fraction by itself into a light aviation base stock boiling essentially within the range of about 90° C. and 155° C. and a heavy fraction boiling essentially within the range of about 140° C. and 200° C., further non-catalytically cracking said heavy fraction, separating the resulting further cracked product by itself to produce an aviation base stock boiling essentially within the range of about 100° C. and 200° C., each of said cracking operations being conducted at a temperature between about 540° C. and 580° C. and at a pressure between about 40 and 100 kg./sq. cm.

9. A process for producing an aviation gasoline base stock from a straight run naphtha having a boiling range essentially within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction in the presence of a minor amount of a light feed consisting essentially of at least one hydrocarbon having from 3 to 5 carbon atoms per molecule, separating the resulting re-cracked product by itself to produce a third naphtha fraction boiling essentially within the range of about 100° C. and 200° C., further separating said third naphtha fraction by itself into a light aviation base stock boiling essentially within the range of about 100° C. and 150° C. and a heavy fraction boiling essentially within the range of about 150° C. and 200° C., further non-catalytically cracking said heavy fraction in the presence of a minor amount of a light feed consisting essentially of at least one hydrocarbon having from 3 to 5 carbon atoms per molecule, and separating the resulting further cracked product by itself to produce a heavy aviation base stock boiling essentially within the range of about 100° C. and 200° C., each of said cracking operations being conducted at a temperature between about 540° C. and 580° C. and at a pressure between about 40 and 100 kg./sq. cm.

10. A process for producing an aviation gasoline base stock from a straight run naphtha having a boiling range essentially within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction in the presence of a minor amount of a light feed consisting essentially of at least one hydrocarbon having from 3 to 5 carbon atoms per molecule, separating the resulting re-cracked product by itself to produce a third naphtha fraction boiling essentially within the range of about 100° C. and 200° C., further separating said third naphtha fraction by itself into a light aviation base stock boiling essentially within the range of about 100° C. and 150° C. and a heavy fraction boiling essentially within the range of about 150° C. and 200° C., further non-catalytically cracking said heavy fraction in the presence of a minor amount of a light feed consisting essentially of at least one hydrocarbon having from 3 to 5 carbon atoms per molecule, and separating the resulting further cracked product by itself to produce a heavy aviation base stock boiling essentially within the range of about 100° C. and 200° C., each of said cracking operations being conducted at a temperature between about 540° C. and 580° C. and at a pressure between about 40 and 100 kg./sq. cm.

11. A process for producing an aviation gasoline base stock from a straight run naphtha having a boiling range within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction in the presence of a minor amount of a light feed consisting essentially of at least one hydrocarbon having from 3 to 5 carbon atoms per molecule, and separating the resulting further cracked product by itself to produce a heavy aviation base stock boiling essentially within the range of about 100° C. and 200° C., each of said cracking operations being conducted at a temperature between about 540° C. and 580° C. and at a pressure between about 40 and 100 kg./sq. cm.

a pressure between about 40 and 100 kg./sq. cm.

10. A process for producing an aviation gasoline base stock from a straight run naphtha having a boiling range essentially within about 90° C. and 230° C., comprising the steps of non-catalytically cracking said naphtha, separating the resulting cracked product by itself to produce a second naphtha fraction boiling essentially within the range of about 90° C. and 230° C., non-catalytically re-cracking said second naphtha fraction, separating the resulting re-cracked product by itself to produce a third naphtha fraction boiling essentially within the range of about 100° C. and 200° C., treating said third naphtha fraction to remove a major portion of olefins therein, further separating said third fraction by itself into a light aviation base stock boiling essentially within the range of about 100° C. and 150° C., and a heavy fraction boiling essentially within the range of about 150° C. and 200° C., further non-catalytically cracking said heavy fraction, separating the resulting further cracked product by itself to produce a heavy aviation base stock boiling essentially within the range of about 100° C. and 200° C., each of said cracking operations being conducted at a temperature between about 540° C. and 580° C. and at a pressure between about 40 and 100 kg./sq. cm.

11. The process of claim 10, wherein the said treating step comprises contacting said third naphtha fraction with between about 1% and 5% by volume of concentrated sulfuric acid and re-distilling the acid treated fraction to remove any polymers formed by the acid.

12. The process of claim 10, wherein said heavy aviation base stock has a boiling range between about 120 and 180° C.

13. The process of claim 10, wherein said heavy aviation base stock is also treated to remove a major portion of olefins therein.

40

14. A process for producing an aviation gasoline base stock from a straight run naphtha having a boiling range essentially within about 100° C. and 200° C., comprising the steps of non-catalytically cracking said naphtha, separating the resulting cracked product by itself to produce a second naphtha fraction boiling essentially within the range of about 100° C. and 200° C., re-cracking said second naphtha fraction in the presence of between about 5% and 30% by volume of a light feed consisting essentially of at least one hydrocarbon having from 3 to 5 carbon atoms per molecule, separating the resulting re-cracked product by itself to produce a third naphtha fraction boiling essentially within the range of about 100° C. and 200° C., treating said third naphtha fraction to remove a major portion of the olefins therein, further separating said treated third naphtha fraction by itself into a light aviation base stock boiling essentially within the range of about 100° C. and 150° C., and a heavy fraction boiling essentially within the range of about 150° C. and 200° C., further non-catalytically cracking said heavy fraction in the presence of between about 5% and 30% by volume of a light feed consisting essentially of at least one light hydrocarbon having from 3 to 5 carbon atoms per molecule, separating the resulting further cracked product by itself to produce a heavy aviation base stock boiling essentially within the range of about 120° C. and 190° C., treating said heavy aviation base stock to remove a major portion of the olefins therein and blending the resulting treated heavy aviation base stock to produce an aviation fuel, each of said cracking operations being conducted at a temperature between about 540° C. and 580° C. and at a pressure between about 40 and 100 kg./sq. cm.

IVOR G. NIXON.